

Sept. 20, 1932.

S. W. YATES

1,878,226

PROCESS OF HEAT TREATING IRON SULPHIDE MATERIAL

Filed April 4, 1928



— 1 —



— 2 —

INVENTOR.

BY *Sampson W. Yates*  
*Allen + Allen*

ATTORNEY.

## UNITED STATES PATENT OFFICE

SAMPSON W. YATES, OF CINCINNATI, OHIO, ASSIGNOR TO THE RICHARDSON COMPANY,  
OF LOCKLAND, OHIO, A CORPORATION OF OHIO

## PROCESS OF HEAT TREATING IRON SULPHIDE MATERIAL

Application filed April 4, 1928. Serial No. 267,309.

My invention relates to the heat treating of iron sulphide materials and particularly ferrous sulphide, so that sound castings can be made of this material; and my process is particularly valuable in connection with electrolytic processes utilizing anodes of ferrous sulphide material. Such an electrolytic process is described in the co-pending application of John R. Cain, Serial No. 238,232, filed December 6, 1927, entitled "Process of plating soft iron".

In accordance with this process soft, malleable and ductile electrodeposits of iron are produced through the use of soluble anodes in a hot neutral ferrous electrolyte such as ferrous chloride. The desired characteristics in the iron deposit seem to be produced at controlled pH values in the electrolyte (in combination with the other factors). The maintaining of an electrolyte under conditions of continuous usage in a ferrous condition and at a desired pH value, i. e. the conditioning of the electrolyte, is a major problem with which the said invention of John R. Cain is concerned; and he has found that anodes of ferrous sulphide material in his process act not only as a source of iron, but also as conditioners to maintain a ferrous condition of the electrolyte and control its hydrogen ion concentration.

It will be seen that for use as anodes in any considerable size, sound castings of the ferrous sulphide materials are requisite. Cracked castings conduct the current poorly and disintegrate unevenly, whereas broken castings are either unusable at all or, if usable, require a plurality of contacts and much expense in handling.

In another application filed herewith and entitled "Processes of producing ferrous sulphide material", in the names of John R. Cain and myself, there is described a method of producing a ferrous sulphide material in a cupola or shaft furnace. One procedure outlined in this application is to crush hema-

ite iron ore, coke and iron pyrite or ferric sulphide of iron and to briquette mixed portions of the material containing the requisite percentages of iron ore, reaction coke and pyrite. The briquettes are treated in a furnace which may be of the ordinary cupola type, and under the influence of heat the hematite iron ore is reduced and the iron combines with an atom of sulphur released by the heat from the ferric sulphide. Molten ferrous sulphide collects in the bottom of the cupola and may be tapped off. My present invention is applicable to the ferrous sulphide material produced by this process or by any other process of producing it in a molten condition; and obviously it will be equally applicable to the casting of ferrous sulphide materials which have been remelted.

Heretofore, while there has been some variation in the iron sulphide product manufactured by the process above referred to and by other processes, such variations depending somewhat upon the nature of the charge and the conditions in the furnace, I have found that the ferrous sulphide materials have a tensile strength generally in the neighborhood of and averaging 450 pounds per square inch.

Further, these ferrous sulphide materials have essentially a smooth cooling curve and also a smooth expansion curve. The expansion and contraction thereof with heat is great, and when the material is taken from the cupola or shaft furnace in a molten condition and poured from a ladle into moulds suitable for the production of anodes, as cooling proceeds there is such a contraction of the outer or cooler layers of the casting while the central part is still quite hot as to cause cracks and fissures to form therein when the two portions, after solidification, approach room temperature. Frequently entire corners will break off the casting, and the casting itself may split into two or more pieces. This action is accelerated by the rapidity of

cooling; but I have not been able to make sound castings of ferrous sulphide excepting by the heat treatment which I shall describe in these specifications.

- 5 As will be clear from what has just been pointed out, the low tensile strength of the material makes it susceptible to cracking from comparatively slight internal strains, and necessitates a heat treatment which will 10 practically neutralize internal strains while increasing the tensile strength. I have developed a heat treatment which will increase the tensile strength practically fifty per cent, and produce a sound casting, free from 15 cracks.

In the drawing:—

- Figure 1 is a reproduction of a micro-photograph at 100 diameters of a representative sample of ferrous sulphide material from an 20 unheat-treated casting.

Figure 2 is a representation of a photograph at the same magnification of a heat treated sample thereof, taken from the same lot and having the same composition.

- 25 It should be pointed out that the applicability of my process is not limited to pure ferrous sulphide (FeS). The iron sulphide material that is made in the cupola or shaft furnace by the process referred to above may 30 contain various percentages of iron and of sulphur, depending upon the charge and the furnace conditions. It is possible that at times a material is obtained which has the approximate formula  $Fe_7S_5$  and that there may 35 also be obtained mixtures of this material with iron or with oxide of iron, or mixtures of FeS with iron or oxide of iron, by the inclusion of an excess of hematite.

- With the proportionate amount of reaction 40 coke and surplus iron in a shaft furnace I may make a material which comprises a percentage of free iron, apparently in solution in ferrous sulphide. There is a possibility that eutectic mixtures are frequently formed; 45 and I have noted that the ferrous sulphide formed under advantageous conditions in the shaft furnace has a melting point lower than ferrous sulphide in a pure state has. This may indicate the presence in solution of 50 oxides of iron and possibly other substances, while at times there may be formed eutectics of oxides and/or iron, and sulphide of iron.

In any event I have found that my heat treating process works with all of the various 55 ferrous sulphide materials, and I have also found that it works very well with mixtures of ferrous sulphide and other materials. My experiments have shown that it is perfectly successful in producing a solid casting comprising 50% ferrous sulphide and 60 50% hematite, which have been melted up together.

While I do not wish to be bound by my 65 present theories respecting the behavior of ferrous sulphide materials in my heat treat-

ing process, I explain this result upon the theory that my heat treatment is effective with ferrous sulphide materials as such and that the soundness of a casting in which I have eliminated disruptive internal strains is not affected by the mere presence in inter-crystalline spaces of extraneous substances such, for example as ferric oxide. I have already pointed out that these ferrous sulphide materials have relatively smooth expansion curves and cooling curves; and so far as I am aware, there are not points at which during cooling sharp crystalline changes occur.

70 The problem is essentially one of the neutralization of the internal strains which result from cooling so that they may be reduced below the tensile strength of the material, and of the closing up of the grain structure as shown in the photomicrographs so as to 75 produce a product of much greater tensile strength.

80 I accomplish the object of my invention by that series of steps which I shall now more fully set forth and claim.

85 I prefer to take the molten ferrous sulphide material from the cupola or shaft furnace or other melting device in the ordinary ladle and to let it remain in the ladle or other container until it has cooled to a temperature 90 close to its freezing point. As it comes from the shaft furnace the material will ordinarily be somewhat superheated. As it cools, it will 95 change from white gradually to yellow, and from yellow gradually to orange. I prefer to 100 cast in the deeper orange phase, if solidification is to be allowed in a mould in the open air.

105 I have found that I may, however, produce sound castings at a pouring temperature ranging from considerable superheat to a point where some crystals have begun to form in the ladle while the main body of the ferrous sulphide material is still fluid. If crystals have commenced to form, of course, solidification is more rapid, the casting must be 110 done rapidly and in ordinary commercial operations it is not possible to control the time in relation to the temperature so closely. Therefore, the material is ordinarily cast at 115 a temperature somewhat higher than that at which crystals begin to form.

120 The molten material is poured into moulds which for my purpose are preferably of cast iron or steel, because of the moderate degree of chilling obtained, although moulds of refractory materials may be used also. They may be in the shape of open pans or they may be in the shape of open top moulds in which the top constitutes one of the narrower sides of the casting. They may be totally enclosed and they may have square corners without fillets. In these moulds the material freezes at a fairly rapid rate, which I desire because 125 it gives a relatively fine crystalline structure 130

and hence forms the casting itself with a maximum of initial tensile strength.

When the casting in the mold is frozen or solidified, I permit it to cool somewhat further, but I do not carry my cooling to the point where cracks begin to occur. Ordinarily I cool until the body of the material is at a bright red heat, a temperature of 1370° F. or thereabouts, and just until the edges begin to darken, whereupon I remove it to a heat treating furnace where the temperature is kept constant at 1100° F. for, roughly, two hours. Following this, the casting is removed to another section of the furnace in which the temperature gradually falls, finally reaching room temperature in from one to one and one-half hours. Some variation in the cooling rate is permissible.

The preferred embodiment of my casting and heat treating process comprises casting at a relatively low temperature and freezing moderately rapidly in the mould, for the purpose of producing a fine grained crystalline structure. In this cooling process the nucleus of some strains will be set up because of the variation in temperature from center to edge of the material, after it solidifies. Before these strains have increased beyond the material's tensile strength, and before the casting has cooled very far I treat it to bring about an equalization of temperature in all its parts. The temperature to which I heat it is such that all strains, including the accompanying temperature equalization strains, will not rupture the material but will themselves be neutralized.

The selection of this temperature is vital. It must be high enough, of course, to bring about such a condition in the material as to permit the neutralization of strains. I believe this to be a point at which the material is slightly plastic. But in addition to this it must not be such as will independently set up strains in the material greater than its tensile strength will stand. A variation beyond certain limits from the optimum temperature, as hereinafter explained, will not produce good results. If the temperature is too low the strains will not be neutralized; if too high, new strains develop upon cooling.

I believe that at the temperature of 1100° F. or thereabouts the ferrous sulphide material is very slightly plastic, i. e. has enough flow to permit these strains to adjust themselves, and I find that such adjustment takes place, roughly, in one and one-half to two hours of heat treatment. During this heat treatment all parts of the casting are brought to the same temperature, and if I thereafter cool carefully so that the temperature fall takes place without excessive variation from center to edge, I find that I produce absolutely sound anodes of any convenient size

for use, such as anodes weighing 100 pounds apiece.

I have made sound castings by heat treatment at 1075° F. but the best results are obtained at 1100° F. The tendency is, if heat treatment is attempted much below 1100° F., for the casting to rupture while in the furnace. If, however, temperatures much above 1100° F. are used for heat treatment, the casting does not crack in the furnace but develops numerous edge cracks on even extremely slow cooling such as in twelve hours. These temperature measurements were made with standard thermocouple apparatus and are of course subject to the usual errors, if any, in apparatus of that type.

It is desirable that the pouring temperature should not be too much above the freezing point because in that case the rate of solidification is slow, and a coarse, weak crystalline structure is obtained. Pouring at a higher temperature with a subsequent chilling in the mould freezes the material quickly, but at the same time sets up so much temperature variation in the casting that the material breaks up before or while the heat treating is being done.

There is, therefore, a maximum amount of superheat that can be tolerated and a more or less definite rate of solidification which is desirable. In my experience this rate is obtained by open air solidification in a mould having walls, roughly, one-half inch thick. If the cast piece is placed in the heat treating furnace too late, so that the temperature of the interior of the casting is much below 1370° F., it breaks up after being placed in the heat treating furnace. Of course, when the body of the casting is at 1370° F., the edges will be somewhat cooler.

The reason for the formation of sudden cracks upon simple cooling seems to be that the outside of the casting, cooling first, contracts while the inside, being warmer, tends to maintain its original size, so that the outer shell is split apart. The reason for the cracking of a casting in the heat treating furnace may be that as the piece is heated up, the temperature equalization sets up strains in the casting some parts of which had cooled below the slightly plastic stage. In any event the casting must be placed in the heat treating furnace before it has cooled too far. By careful dilatometer tests, I have found the coefficient of expansion of the iron sulphide material to be, roughly, three times that of iron, which fact, when considered in connection with its relatively very low tensile strength indicates the magnitude of the problem solved by my heat treating process in the production of sound castings.

While the casting is in the heat treating furnace at 1100° F., the whole is brought to a uniform temperature and all strains are apparently released. The material, I believe,

is at this temperature very slightly plastic so that the strains can produce slight deformations. The material also seems to become of closer grain, denser and much tougher.

6 After the heat treating process it must not be chilled too quickly or the unequal temperature in various parts will set up enough new strains to rupture the material.

If an unheat-treated, cold sample is slowly 10 brought up to 1100° F., and then allowed to cool slowly, numerous cracks develop on cooling from the edges toward the center. This is because the material is not strong enough

15 to stand the strains set up by deformation due to differences in temperature between center and outside as the material cools. My heat treating process, however, puts the material into such condition and makes it so strong that it can be cooled down fairly rapidly without any cracking, as I have before indicated.

I have found that by removing the mould and the casting together from the furnace to the open air in moderate weather and in the 25 absence of drafts, with the open top covered by a steel plate, a sound casting can be produced; but for commercial operation where it is not advisable to take any chances of the cracking of anodes, it is advisable, as I have already indicated, to place the casting in a portion of the furnace where the temperature gradually falls from 1100° F. to room temperature in an hour or possibly more.

After my heat treatment, I have found that 25 the average strength of the ferrous sulphide material (and by this I mean material consisting almost wholly of ferrous sulphide of iron) is increased from 450 pounds per square inch to 675 pounds per square inch, an increase of 50%. It resists breaking with a hammer much better, and is strong enough to be handled in large, thin slabs. The heat treated material appears closer grained, denser and tougher, as will be seen in the microphotographic representations forming 45 Figures 1 and 2 of the drawing. It is possible that other changes take place in the material, which I have not yet determined by experiment, such possibly, as an actual increase in specific gravity and a contraction in volume.

Heat treating furnaces for the accomplishment of my purpose are within the capabilities of those skilled in the art to construct. 55 They may be of various forms, as will be clear, and my process may be somewhat varied in different types of heat treating furnaces without departing from the scope of my invention.

60 Having thus described my invention, what I claim as new and desire to secure by Letters Patent, is:—

1. A process for obtaining sound castings of a material comprising ferrous sulphide, 65 which comprises casting said material and

permitting solidification thereof in a mould and thereafter, without permitting said solidified casting to cool until internal strains set up by said solidification and cooling become greater than the tensile strength of said casting so as to cause cracks therein, subjecting the said casting to a degree of temperature short of the liquefaction point but sufficient to render it slightly plastic, for a sufficient time to permit the neutralization of internal strains and the closing up of grain structure, and then cooling said casting slowly and evenly to room temperature.

2. A process for obtaining sound castings of a material comprising ferrous sulphide, which comprises casting said material at a temperature close to its freezing point and permitting the quick solidification thereof in a mould so as to obtain a fine grain of crystallization in the casting, and thereafter, without permitting said casting to cool until internal strains set up by said solidification and cooling become greater than the tensile strength of said casting so as to produce cracks therein, subjecting said casting to a degree of heat short of the liquefaction point thereof but sufficient to render it slightly plastic for a period of time sufficient to permit the neutralization of internal strains, and the improvement in grain structure resulting in greater strength, and then cooling said casting at a rate such that a substantial uniformity of temperature is maintained throughout it.

3. A process of obtaining sound castings 100 of a material comprising ferrous sulphide, which comprises casting said material and allowing it to cool rapidly while freezing to a temperature above 1300° F., at the center, then transferring the casting to a heating zone and there maintaining it at a constant temperature higher than 1000° F. but below its liquefaction point for about two hours, then cooling said casting evenly to room temperature in about one hour.

4. A process for obtaining sound castings in a material comprising ferrous sulphide, which comprises cooling said material before casting until it becomes a deep orange, casting said material while still molten, and allowing it to cool rapidly in the moulds while freezing to a temperature at which the body of said material is at a bright red heat and the edges thereof begin to darken, then placing said casting in a heat treating zone and there maintaining it at a constant temperature higher than 1000° F. but below its liquefaction point for about one and one-half hours, then cooling said casting evenly to room temperature in not less than one hour.

5. A process for obtaining sound castings of a material comprising ferrous sulphide, which comprises cooling said material in a ladle to a temperature just above its freezing point, casting said material into metallic

moulds in the open air and permitting it to cool therein until solidified and until it reaches a temperature around 1370° F., thereupon transferring the casting to a heat treating furnace and maintaining it there for not less than one and one-half hours at a temperature of 1100° F., then cooling said casting evenly to room temperature in not less than one hour.

10 6. A sound casting of a material consisting essentially of ferrous sulphide, said casting having as the result of a heat treatment a tensile strength at least 675 pounds per square inch.

15 SAMPSON W. YATES.

20

25

30

35

40

45

50

60

65